

## UNITED STATES PATENT OFFICE

2,304,242

## DIESEL FUEL

Gould H. Cloud, Elizabeth, N. J., assignor to  
Standard Oil Development Company, a corpora-  
tion of Delaware

No Drawing. Application March 22, 1939,  
Serial No. 263,407

6 Claims. (Cl. 44—9)

This invention relates to a stabilization of compression-ignition engine fuels and is concerned particularly with improved fuel compositions adapted for high speed engines of the Diesel type by addition compounds which enhance ignition qualities of the fuel.

In most instances, addition compounds which have been recommended for accelerating ignition of hydrocarbon oils in Diesel engines have characteristically contained oxygen, nitrogen, and sulfur, in highly unstable groupings. While it is true that many of these proposed compounds are very effective in shortening the delay period between injection and spontaneous ignition of the fuel, particularly when the fuel is freshly made up, a reduction in their effectiveness tends to occur during storage owing to their inherent instability. Not only do these unstable compounds tend to deteriorate, but on deteriorating they tend to induce oxidation of hydrocarbons in the fuel which results in gum formation and further, they tend to develop corrosive decomposition products in storage and in operation of the engines.

The object of this invention is to provide an improved Diesel fuel composition with a novel stabilizing agent, which, added to the fuel by itself or in combination with unstable types of ignition promoters, has a definite and substantial beneficial influence on the ignition quality of the fuel.

Compounds suitable for use as stabilizing promoters according to the present invention are certain organic nitrogen compounds characterized by having adequate solubility in hydrocarbon oil and chemical properties which adapt them for inhibiting oxidation and corrosion. Compounds responding to these requirements were found to be notably hydrazines, certain hydrazine derivatives, and certain related nitrogen bases. These compounds behave exceptionally well in enhancing the qualities of Diesel fuel oils, since, in general, the presence of an amino or an imino group in a compound has appeared to counteract ignition-promoting action generally, for example, aromatic amines, e. g., aniline, and their usual derivatives, including azo and hydrazo compounds, have been determined to be detrimental to the ignition qualities of a fuel.

Hydrazines which are used in the practice of this invention belong to a well known class of unsymmetrical compounds identified by the presence of nitrogen in the groupings —NH·NH<sub>2</sub>,

—N.NH,

and —NH·NH—. Members of this class of compounds found to be preferably useful are dimethyl hydrazine, phenyl hydrazine, diphenyl hydrazine, and methyl phenyl hydrazine—in

each instance, the methyl and phenyl groups being replaceable by higher homologous hydrocarbon radicals. Similarly suitably hydrazine derivatives and related nitrogen bases are quinu-  
5 alyl hydrazine, acetyl phenyl hydrazine, 3-amino phthal hydrazine, carbazole, 5-amino uracil, and tribenzyl amine.

The manner of employing the compounds which possess desirable properties for promot-  
10 ing qualities and stability in Diesel fuels and of testing their efficacy in these respects is illus-  
trated in the following description.

A number of samples were prepared by dis-  
solving from less than 1% to about 3% by vol-  
15 ume of the compound to be tested in a portion  
of a 40 cetane number gas oil, and each sample  
was tested in a high speed Diesel engine acc-  
cording to the method disclosed in the S. A. E.  
Journal of June, 1936, page 225. Each sample  
20 was rated on its cetane number by compari-  
son with blends consisting of cetane and alpha-meth-  
yl naphthalene. Since the ignition lag of a blend  
consisting of normal cetane and alpha-methyl  
naphthalene is shortened very nearly in propor-  
25 tion to the increase in percentage of cetane by  
volume, the ignition quality of a fuel can be  
evaluated in terms of the cetane content of such  
a blend giving comparable performance in the  
test engine.

Even though a number of aliphatic amines,  
30 aromatic amines, and their derivatives consist-  
ently showed an adverse effect on the cetane  
number of the fuel samples, the dialkyl, diaryl,  
and alkyl-aryl hydrazines and hydrazine deriva-  
35 tives, particularly those enumerated, made a sub-  
stantial improvement in the cetane number of  
the fuel. The compounds selected as preferable  
are those which increase the cetane number of  
a fuel on the order of 2 or more points when in-  
40 corporated in concentrations of less than about  
1% by volume of the fuel. Further tests on fuel  
samples blended with mixed ignition promoters  
show that by using the compounds capable of  
45 promoting and stabilizing ignition qualities of the  
fuel together with addition compounds having  
higher potency for accelerating ignition but lack-  
ing stability, the ignition qualities of the blend-  
ed fuel is increased at least in proportion to the  
50 effect of each promoter. Considerable impor-  
tance is attached to this fact, because ignition  
promoters are closely in comparison to the value  
of hydrocarbon fuels, making it highly desirable  
55 to eliminate any detrimental influence of pro-  
moters without impairing their ignition acceler-  
ating action.

To prepare the Diesel fuel compositions which  
can be stored for long periods without detriment  
to the ignition qualities, also with reduced acid  
60 and sludge formation, the ignition promoting

stabilizing compound need be used only in less than about 1%, whether used alone or together with .5% to about 5% of addition compounds such as aromatic peroxides, aliphatic nitrates, aliphatic nitrites, aliphatic polysulfides, and the like. About .2% to 1% of the stabilizing promoter is generally adequate, but with more readily oxidizable fuels or more unstable addition compounds as much as 3% may be used.

Every hydrocarbon oil suitable as a fuel for Diesel engines may be improved in the described manner. Ordinarily, the hydrocarbon fuel to be used may be said to have a boiling range above that of gasoline, and, more particularly, the boiling range and viscosity of hydrocarbons present in a gas oil which boils from 400° F. to 700° F. Under some circumstances, a more narrowly cut fraction such as one distilling from about 400° F. or 450° F. to 600° F. may be used. Considerable benefits are obtained in improving lower cost fuels by the stabilizing promoters in that the lower cost fuels contain large quantities of hydrocarbons unstable toward oxidation.

Small quantities of the novel addition agents of this invention are useful for adapting various mixtures of hydrocarbons for use as Diesel fuels, including recycle stocks from cracking operations, non-paraffinic extracts, distillates from the destructive distillations of coal and asphaltic materials, and mixtures of these with one another or with crude petroleum fractions. Other agents for enhancing various other qualities without detracting substantially from the ignition qualities of the fuel may be admixed, such as oiliness agents, dyes, pour point depressants, and viscosity modifiers.

Practical advantages obtained in using the stabilizing promoters are:

1. Economy in the use of more potent ignition promoters which are subject to degradation when used without a stabilizing agent;
2. Protection of storage tanks and engine parts from corrosive decomposition products of the more potent ignition promoters;

3. Stabilization of the fuel against the development of insoluble gums and resins which tend to clog fuel lines and atomizers; and

4. Elimination of substances having harmful and annoying physiological effects from exhaust gases.

The above description and examples are to be taken as illustrative only and not as limiting the scope of the invention. Any modification or variation therefrom which conforms to the spirit of the invention is intended to be included within the scope of the claims.

I claim:

1. A compression-ignition engine fuel comprising a hydrocarbon oil boiling from 400° F. to 700° F. and as an ignition improver and stabilizing agent a minor amount of an essentially hydrocarbon unsymmetically substituted hydrazine compound selected from the group consisting of dialkyl hydrazines, phenyl hydrazine, diaryl hydrazines, alkylaryl hydrazines, quinalyl hydrazine, acetyl phenyl hydrazine, 3-amino phthal hydrazine.

2. A fuel composition as described in claim 1 having admixed therewith a minor amount of an ignition accelerating agent selected from the class consisting of aliphatic nitrates, aliphatic nitrites, aromatic peroxides, and aliphatic polysulfides.

3. A compression-ignition engine fuel comprising a hydrocarbon Diesel fuel oil and as an ignition improver and stabilizing agent a minor amount of an unsymmetrical hydrazine containing a hydrocarbon substituent radical.

4. A compression-ignition engine fuel comprising a hydrocarbon Diesel fuel oil and .2% to 1% of phenyl hydrazine.

5. A compression-ignition engine fuel comprising a hydrocarbon Diesel fuel oil and .2% to 1% of methyl phenyl hydrazine.

6. A compression-ignition engine fuel comprising a hydrocarbon Diesel fuel oil and .2% to 1% of an unsymmetrical essentially hydrocarbon diaryl hydrazine.

GOULD H. CLOUD.